

## UNITED STATES PATENT OFFICE

CARL DANKERT, OF LUDWIGSHAFEN-ON-THE-RHINE, GERMANY, ASSIGNEE TO I. G. FARBEININDUSTRIE AKTIENGESELLSCHAFT, OF FRANKFORT-ON-THE-MAIN, GERMANY

## COLORED EFFECT PAPER

No Drawing Application filed November 24, 1931, Serial No. 577,151, and in Germany November 28, 1930.

The present invention relates to colored effect papers and process of producing same.

I have found that beautiful colored effect papers are readily obtained on the paper machine by supplying to the paper pulp on the sieve near to the gate a solution of a water-insoluble cellulose derivative in an organic solvent. The said solution may be supplied in the form of drops or jets by the well-known devices, such as nozzles or containers arranged above the sieve and containing small openings in the bottom. Water-insoluble cellulose derivatives which may be used for the present purpose are cellulose esters, such as for example nitrocellulose and cellulose acetate, propionate and butyrate and cellulose ethers, for example ethylcellulose and benzylcellulose. The said cellulose derivatives may be dissolved in the known solvents or mixtures thereof, such as for example acetone, alcohols, such as methyl and ethyl alcohol, and their esters, for example butyl acetate, vinylacetate, benzene and its homologues, benzine, cyclohexanone, cyclohexanol and their homologues and the like. Particularly suitable for dissolving nitrocellulose are mixtures of solvents containing acetone. Softeners or plasticizers may be added to the solutions of the cellulose derivatives, for example castor oil, diethylphthalate, triphenylphosphate, tricresylphosphate, diacetin, triacetin and the like.

In order to produce colored effect paper with the aid of the said solutions of cellulose derivatives either the latter or the paper pulp or both the cellulose derivative solution and the paper pulp are colored by means of dyestuffs or pigments. Any dyestuffs or pigments may be used for the said purpose.

When introducing the said solutions of cellulose derivatives into the paper pulp, the cellulose derivatives are precipitated from their solutions and form a kind of thin film on the paper pulp covering the paper pulp wholly or in places. In order to completely precipitate the cellulose derivative from its solution it is necessary that sufficient water is still present in the pulp. This is the case when the paper pulp passes the gate on the wet-part of the paper machine and, therefore,

the solution of the cellulose derivative is added to the pulp near the gate or if such is not provided in the paper machine at the point where the paper pulp contains a corresponding amount of water.

In order to produce particular effects soap solutions, ether or ox gall may be supplied to cellulose derivative film formed.

The following examples will further illustrate how the invention may be carried out in practice, but the invention is not restricted thereto. The parts are by weight.

## Example 1

10 parts of nitrocellulose are dissolved in a mixture of 175 parts of acetone, 0.5 part of castor oil, 0.5 part of colophony, 300 parts of ethyl alcohol, 100 parts of toluene and 20 parts of benzine. Part of this solution is colored by means of Indanthren red BN (Colour Index, 1924, No. 1162), a second part with Sudan brown (Colour Index, 1924, No. 81) and a third part with Indanthren blue 3G (Colour Index, 1924, No. 1109), or with ultramarine (Colour Index, 1924, No. 1290). The said colored solutions of nitrocellulose are then dropped, or slowly run, side by side, into the paper pulp near the gate. On the surface of the paper red, brown and blue films are formed and a marbled paper is obtained.

## Example 2

10 parts of nitrocellulose are dissolved in a mixture of 20 parts of butyl acetate, 325 parts of acetone, 0.5 part of tricresyl phosphate, 0.5 part of polyvinylacetate, 120 parts of ethyl alcohol, 30 parts of toluene and 2.2 parts of benzine. The solution is colored with Paris blue (Colour Index, 1924, No. 1288) and is allowed to run on to the paper pulp in the manner described in the foregoing example.

The nitrocellulose solution may also be colored by means of copper or aluminium bronze.

## Example 3

10 parts of film chips are dissolved in a mixture of 200 parts of acetone, 70 parts of ethyl alcohol, 35 parts of toluene, 2 parts of

benzine and 1 part of butyl acetate. The said solution is run near the gate on to paper pulp stained with cotton black (Colour Index, 1924, No. 581 or 582).

In order to produce more contrasted effects the solution of nitrocellulose may be colored with blanc fix or titanium white (Colour Index, 1924, No. 1264).

What I claim is:

1. A process of producing colored effect papers on the paper machine which comprises supplying to the paper pulp on the sieve near the gate a solution of a water-insoluble cellulose derivative in an organic solvent, at least one of the said components forming the effect paper being colored.

2. A process of producing colored effect papers on the paper machine which comprises supplying to the paper pulp on the sieve near the gate a colored solution of a water-insoluble cellulose derivative in an organic solvent.

3. A process of producing colored effect papers on the paper machine which comprises supplying to the paper pulp on the sieve near the gate a colored solution of nitrocellulose in an organic solvent containing acetone.

In testimony whereof I have hereunto set  
30 my hand.

CARL DANKERT.

35

40

45

50

55

60

65